

July 15, 1941.

L. C. GALATIOTO

2,249,607

METHOD OF DYEING CELLULOSE ACETATE AND DYE BATH COMPOSITIONS

Filed April 24, 1939

300/100/3 BRIGHT ACETATE YARN DELUSTERING TESTS



BATH COMPOSITION PERCENTAGE BY WEIGHT

|                   | H     | V      | F      | E      | W  | X  |
|-------------------|-------|--------|--------|--------|----|----|
| ○                 | ○     | △      | □      | ◊      | Λ  | —  |
| 85% ACID FORMIC   | 8 1/3 | 8 1/3  | 16 2/3 | 10     | 5  |    |
| 84% ACID ACETIC   | 8 1/3 | 8 1/3  | 8 1/3  | 16 2/3 | 10 | 5  |
| 20° Be' SULPHURIC | 8 1/3 | 8 1/3  | 8 1/3  | 8 1/3  | 10 | 5  |
| WATER             | 75    | 83 1/3 | 83 1/3 | 83 1/3 | 70 | 85 |

NOTE—AREA ABOVE GRAPH LINE—DELUSTERING  
AREA BELOW GRAPH LINE—NON DELUSTERING

Inventor,  
Luis C. Galatioto  
by John Bushman, Notary  
his Atty.

## UNITED STATES PATENT OFFICE

2,249,607

METHOD OF DYEING CELLULOSE ACETATE  
AND DYE BATH COMPOSITIONSLuigi C. Galatioto, Providence, R. I., assignor to  
Atlantic Rayon Corporation, Providence, R. I.  
a corporation of Rhode Island

Application April 24, 1939, Serial No. 269,661

24 Claims.

(Cl. 8—59)

The present invention relates to a method of dyeing cellulose acetate, in its various forms, such as yarn, woven fabrics, films, sheets or the like, and to dye bath compositions of suitable characteristics for carrying out the method.

Cellulose acetate, as originally made, was obtained by the complete acetylation of cellulose to form the tri-acetate or tri-acetyl cellulose. This product was utilized for a considerable period for various purposes, but it was repellent to water and to liquids generally and accordingly presented many serious difficulties in dyeing. Subsequently, it was found that by first acetylating cellulose to the tri-acetate and then partially hydrolyzing back the acetylated compound, a product was obtained which was softer, more susceptible to wetting with liquids, including water, and which, with some dyes, could be colored. But the color was not fast.

This acetylated and partially hydrolyzed product is technically known as "secondary acetate" and is the product now made and used practically exclusively as "cellulose acetate." It is this product which forms the subject matter to be treated and dyed by the present process, as set forth in the following disclosure.

It is therefore an object of the present invention to provide a method of procedure and suitable reagent solutions and dye bath compositions, which shall render it possible to dye present-day cellulose acetates and the various products which may be made from them—such as fibers, yarns, fabrics, films, sheet materials, granules, coatings, and the like—with acid dyes, to a satisfactory range of colors and color values (such as those of the Standard Color Card of America) on a practicable basis for commercial operations and results. It is also an object to provide a method and dye bath compositions which may be definitely relied upon to dye the goods under treatment effectively, and fast to washing and to light, and to a controllable degree of depth of color, including both dark and light shades, with a pleasing quality of appearance, etc.—and at the same time to retain the desirable qualities of the original "secondary" cellulose acetate such as tensile strength, elongation, luster, feel, lay of the fibers, smoothness of surface, etc. Other objects of the invention will appear from the following disclosure.

It is now found that cellulose acetate as at present made and sold on the market in various forms—which is the "secondary acetate" as above pointed out—may be satisfactorily and permanently dyed with acid dyes, provided certain conditions are developed and maintained with reference to the material under treatment, and to the dye bath and dyeing operations.

It is a common property of cellulose—which is 60 natural fibers. Since it contains one or more

generally recognized with free cellulose fibers in the form of paper—that it spontaneously takes up by adsorption and retains about 7 to 8% of moisture, by weight, even from a normally moist atmosphere. Such adsorption appears to be mechanical, rather than chemical, and the adsorbed moisture is retained upon the surfaces, since no swelling is observed to accompany the gain or loss of this moisture.

10 It is now observed that cellulose acetate, of the type under consideration, manifests a similar adsorption when immersed in water. With cellulose acetate in the form of a sheet—no appreciable change in the dimensions of the sheet is observed either upon adsorption or expulsion of this amount of water, which is about 7% by weight. It may, therefore, be considered as a mechanical adsorption of water by the cellulose acetate surfaces. It is thought that this adsorbed 15 water may associate itself with the cellulose component of the cellulose acetate molecule, upon the free surfaces, analogous to the adsorption of water by free cellulose itself, above mentioned. Additional mechanical associations with water 20 may also occur, however, which are attributable to the porosity of the sheet and the corresponding volumes of the interstices therein as well as adsorption on free surfaces. This is indicated by the fact that cellulose acetate films from different 25 sources exhibit varying degrees of preliminary adsorption.

Similar moistening of cellulose acetate yarn may in some instances be accompanied by an 30 apparent increase in dimensions as indicated by a slight elongation of the material, upon wetting. But such increase is slight and may be attributable to the release of surface tension of the dried 35 surfaces or to slight slippage of the moist fibers over one another, rather than due to swelling 40 effects of moisture upon the individual fibers.

Moreover, capillary attraction between the 45 fibers enters into the wetting of cellulose acetate yarns upon immersion in water, so that the mechanical adsorption and absorption manifested by them (under conditions mentioned hereinafter) is of the order of 42% by weight, in contrast to 7%, by weight, mentioned above with reference to sheet materials.

50 It is necessary to remember that cellulose acetate, in whatever form it is regarded for the purposes of the present consideration, has been hydrolyzed back from the naturally hard water resistant form of the tri-acetyl cellulose to a lower degree of acetylation. Consequently this product 55 is chemically different from other artificially prepared cellulosic fibrous materials (which more closely resemble hydrocellulose) and is both chemically and structurally different from natural fibers. Since it contains one or more

acetyl groups it is subject to further saponification and hydrolysis under alkaline conditions, with further loss of such acetyl groups, on the one hand; and on the other, it is subject to esterification by combination with additional acidic groups, under sufficiently acidic conditions. But further saponification or hydrolysis tends to swell it and render it less desirable, since the physical and dyeing properties are altered. Further esterification—e. g. to the tri-acetate—would render it more resistant to wetting by water solutions.

Nevertheless, partially hydrolyzed or secondary cellulose acetate is soluble in various organic solvents, and many of these solvents are, in turn, soluble in water. A series of water solutions of such solvents, containing increasing concentrations of such solvents, may be prepared and applied to the acetate, with varying effects accordingly. In very low concentrations, such solutions resemble water alone, as would be expected, and have no effect. But with increasing concentrations of the solvent, in aqueous solution, (depending somewhat upon the specific solvent in question) there is a "threshold" point at which such solvent solutions appear to penetrate the cellulose acetate much more readily than water and ultimately to diffuse through it completely, without any tendency to swell or disintegrate it. The first observable effect of treating cellulose acetate with solvent solutions of increasing concentrations is that with each solvent a concentration will be reached at which the cellulose acetate treated therewith loses its brilliant surface luster. This effect is referred to as "de-lustering," and indicates that the surface of the acetate has been affected, at least sufficiently to alter its optical characteristics in respect of the uniform reflection of light. Such concentration of solvent, therefore, is a "critical point" in such treatment, with reference to cellulose acetates to be dyed. Upon further increasing the concentration of the solvent solution it will be found that it will later reach a point at which the absorption from the solution by the acetate treated therewith undergoes an abrupt increase in proportion, by weight. The cellulose acetate also gives evidence of exercising a more retentive absorption of the aqueous solvent solution at this point, and swells. Increasing the concentration of solvent, therefore, leads to a solution which is capable of effecting first a very definite attack upon and finally a disintegration of the cellulose acetate, which may involve first a shrinkage, in over-all dimensions, followed by dispersion of the same and ultimately complete dissolution of the acetate, as is accomplished, for example, by the pure solvent itself.

While specific data, with reference to a given solvent, will vary from that for another solvent or solvents, it may nevertheless be stated that in general aqueous solutions of solvents of cellulose acetate are characterized, in increasing concentrations, by three successive stages;

(1) A "threshold" concentration at and above which the solution exhibits a wetting and penetrating capacity toward the cellulose acetate which is markedly greater than that of water, but without other alterations;

(2) A critical de-lustering concentration, at 70 which the solution causes an alteration in the optical properties of the surface of the cellulose acetate, whereby its reflection of light or "lustre" is noticeably affected or diminished, and the acetate is said to be "de-lustered" but otherwise 75

the material is not substantially changed; and

(3) A critical swelling concentration, at which the solution exhibits a tendency to cause the acetate to undergo marked increase of absorption and to swell, and above which disintegration and ultimately complete dispersion or dissolution of the acetate ensue. (See Table 1.)

#### EFFECTS OF TIME AND TEMPERATURE

It is further found that, with any given solvent solution, of fixed concentration, the percentage of absorption of the solution by the cellulose acetate (by weight) first very rapidly increases to a maximum, and then decreases, and again increases, ultimately exceeding the first maximum, as the period of time of immersion in the solution is progressively increased. (See Table 2.) Also, that the percentage of absorption (by weight) similarly first very rapidly increases and then decreases and again increases as the temperature of the solvent solution used is progressively increased. (See Table 3.) In some cases a tendency to shrink in dimensions also may be observed under these conditions. Accordingly, there is a tendency for a continuously wetted and/or heated acetate, in contact with an aqueous solution of one or more of its solvents, to reach a point where it tends to resist further absorption or even to expel absorbed solution and to contract in its over-all dimensions.

Since the use of solvent solutions of increased concentrations tends so greatly to control the increase of absorption of the solution by the acetate,—the opposite effects of increased time and/or temperature of treatment (which in the present dyeing operation are usually standardized or fixed) are in general overcome or subordinated by the control or selection of the concentration of the solvent solution. But these tendencies of time and temperature apply to solutions of high concentrations of solvent as well as to the more dilute solvent solutions, and are extremely important, as will be pointed out below.

Results of experiments carried out upon cellulose acetates from various sources in the form of thin films, with solvent solutions of increasing concentrations are set forth in the following table:

50  
55

TABLE 1

Percentage increase in weight and length of various films<sup>3</sup> in formic acid

| Concen-<br>tration of<br>formic<br>acid, cal-<br>culated as<br>85% (in<br>water) | Celanese <sup>4</sup><br>Corporation<br>Bright<br>acetate | Viscose<br>Co. <sup>5</sup> cel-<br>lulose<br>acetate | Eastman <sup>3</sup><br>dull ace-<br>tate<br>rayon (1) | Du Pont<br>Co. <sup>3</sup><br>Bright<br>Acetate | Du Pont<br>Co. <sup>3</sup> Dull<br>Acetate (1) |
|----------------------------------------------------------------------------------|-----------------------------------------------------------|-------------------------------------------------------|--------------------------------------------------------|--------------------------------------------------|-------------------------------------------------|
| 5%-----                                                                          | 18.1<br>20                                                | 9.2<br>0                                              | 8.5<br>2.3                                             | 6.4<br>0                                         | 8.8<br>1.0                                      |
| 10%-----                                                                         | 8.4<br>0                                                  | 12.1<br>0                                             | 12.1<br>1.2                                            | 9.8<br>4.1                                       | 11.2<br>1.0                                     |
| 15%-----                                                                         | 12.9<br>1.3                                               | 15.3<br>0                                             | 14.1<br>3.4                                            | 11.8<br>4.1                                      | 14.9<br>4.6                                     |
| 20%-----                                                                         | 15.1<br>7.9                                               | 18.9<br>12.1                                          | 17.0<br>8.0                                            | 15.2<br>4.4                                      | 19.6<br>3.9                                     |
| 25%-----                                                                         | 19.3<br>6.2                                               | 19.3<br>4.8                                           | 17.5<br>5.7                                            | 16.9<br>3.4                                      | 18.1<br>6.8                                     |

Time: 30 min. Temp.: 125° F.

<sup>1</sup> Weight changes, top figures.

<sup>2</sup> Length changes, bottom figures.

<sup>3</sup> These films were obtained by dissolving the named yarn in acetone and casting films upon a glass plate by the usual technique.

<sup>4</sup> Loss.

These results show that aqueous solutions of formic acid of increasing concentrations cause in general a continuously increasing absorption of the cellulose acetate films treated therewith, accompanied by increasing dimensions (elongation) of the films. Also that some films may take up 8-15%, by weight of solvent, without corresponding increase in dimensions—or even with a subsequent appreciable decrease in dimensions.

The effects of varying the "time" of immersion of the acetate in the solvent solution (of various concentrations) at constant temperature—125° F.—will be shown from the following table:

TABLE 2

Percentage increase in weight and length of celanese film in formic acid

|                                           | Time factor       |                    |                    |                    |
|-------------------------------------------|-------------------|--------------------|--------------------|--------------------|
|                                           | 5 min.<br>125° F. | 10 min.<br>125° F. | 30 min.<br>125° F. | 60 min.<br>125° F. |
| Water alone.                              |                   |                    | { 7.2              |                    |
| Formic acid (calculated as 85% solutions) |                   |                    | { 0                |                    |
| 5%                                        | 19.7              | 6.8                | 8.1                | 8.0                |
|                                           | 21.1              | 1.2                | 0                  | 1.1                |
| 10%                                       | 11.1              | 10.9               | 8.4                | 8.7                |
|                                           | 1.1               | 1.2                | 0                  | 1.2                |
| 15%                                       | 15.0              | 13.0               | 12.9               | 11.7               |
|                                           | 1.1               | 1.1                | 1.3                | 2.2                |
| 20%                                       | 18.1              | 16.8               | 15.1               | 14.7               |
|                                           | 7.9               | 8.1                | 7.9                | 9.0                |
| 25%                                       | 22.0              | 20.0               | 19.3               | 17.2               |
|                                           | 7.9               | 6.1                | 6.2                | 5.6                |

<sup>1</sup> Weight changes, top figures.

<sup>2</sup> Length changes, bottom figures.

The effects of varying the temperature of various concentrations of the solvent solution, in which the acetate is immersed for a given period of time (30 minutes), is shown by the following table:

TABLE 3  
Percentage increase in weight and length of celanese film in formic acid

| Formic | Temperature factor |                   |                    |                    |                    |
|--------|--------------------|-------------------|--------------------|--------------------|--------------------|
|        | 30 min.<br>60° F.  | 30 min.<br>90° F. | 30 min.<br>125° F. | 30 min.<br>150° F. | 30 min.<br>180° F. |
| 15     |                    |                   |                    |                    |                    |
| 5%     | { 11.7             | 9.9               | 8.1                | 5.0                | 5.1                |
|        | { 11.2             | 1.1               | 0                  | 0                  | 1.2                |
| 10%    | 15.7               | 8.1               | 8.4                | 7.8                | 7.7                |
|        | 2.2                | 1.2               | 0                  | 0                  | 5.9                |
| 15%    | 20.7               | 14.8              | 12.9               | 10.5               | 9.9                |
|        | 2.4                | 1.1               | 1.3                | 0                  | 7.1                |
| 20     | 25.3               | 18.5              | 15.1               | 13.8               | 15.5               |
| 20%    | { 3.3              | 2.4               | 7.9                | 5.7                | 2.3                |
|        | 29.5               | 24.4              | 19.3               | 18.3               | 21.6               |
| 25%    | 13.0               | 8.9               | 6.2                | 1.1                | 0                  |

<sup>1</sup> Weight changes, top figures.

<sup>2</sup> Length changes, bottom figures.

<sup>3</sup> Loss.

Analogous data for cellulose acetate "yarn" is given in the following table, with increasing concentrations of the aqueous solutions of various cellulose acetate solvents—with indications of whether or not the solvent solution of any particular concentration in question has de-lustered the yarn and hence equals or exceeds the critical point with respect to de-lustering. All of these samples of acetate yarn were liberated from excess of the solvent solution by uniform treatment in the centrifuge to give comparable results. It should be noted that the yarn manifested an initial mechanical absorption of water of 41.9% by weight (under the conditions hereafter described) and that all of the solvent solutions used upon the acetate had the effect of increasing the absorptivity figure.

TABLE 4

Absorption of dye bath by cellulose acetate yarn  
in percent of bone-dry weight of yarn

| Percent of reagent (by volume) | 80% acetic (by weight) | 85% formic (by weight) | 1/2 acetic<br>1/2 formic | 85% lactic (by weight) | 100% ethylene chlorhydrin | 100% acetone | Conditions                    |
|--------------------------------|------------------------|------------------------|--------------------------|------------------------|---------------------------|--------------|-------------------------------|
| 5                              | 44.80 K.               | 52.30 K.               | 46.10 K.                 | 47.6vSL.               | 53.30 K.                  | 45.70 K.     | 300/100/3 Bright              |
| 10                             | 43.70 K.               | 55.0SL.                | 46.6SL.                  | 47.6 SL.               | 56.6Bad                   | 46.90K.      | Acetone (skein 2 oz.) 30 min. |
| 15                             | 53.8SL.                | 64.2Bad                | 47.6Bad                  | 46.3 SL.               | 60.9Bad                   | 49.35L.      | 125° F.                       |
| 20                             | 52.5Bad                | 47.9Bad                | 53.8Bad                  | 56.8 SL.               | 83.2Bad                   | 49.2Bad      |                               |
| 25(A)                          | 52.9Bad                | 53.3Bad                | 51.2Bad                  | 59.9 SL.               | 101.0Bad                  | 49.3Bad      |                               |
| 30(B)                          | 62.6Bad                | 57.3Bad                | 57.5Bad                  | 59.6 SL.               | 122.0Bad                  | 50.7Bad      |                               |
| 40                             | 79.9Bad                | 93.0Bad                | 86.2Bad                  | 69.1 SL.               | (?)                       | 64.9Bad      |                               |
| 50                             | 137.1Bad               | 123.3Bad               | 157.3Bad                 | 81.9Mod.               | (?)                       | 196.9Bad     |                               |

Comments refer to effect on luster:

OK.—luster unaffected.

vSL.—luster very slightly affected.

SL.—luster slightly affected.

Mod.—luster moderately affected.

Bad.—luster badly affected.

—skein badly attacked.

—skein too badly attacked to extract in centrifuge.

(A) No dye used in dye bath solution.

(B) Bone-dry weight determined on separate skeins from those used in the dye baths.

It will be noted from these results that an aqueous solution of solvent, having a concentration of 5% or more has the effect of enhancing the absorptivity of the acetate above that of water alone (41.9%). Also, that this increase of absorptivity continues with solutions of increasing concentration of solvent, but that it generally ceases to increase or even declines at the higher concentrations and then resumes its effect of increasing absorptivity up to the point of disintegration or dissolution of the acetate by the highly concentrated solutions of solvent.

In respect of increasing concentration of the various solvent solutions used, therefore, the "threshold" concentration of aqueous solutions of solvents of cellulose acetate may be taken as approximately 5%.

It is to be observed, however, that the "critical point" with respect to "de-lustering" of the yarn, varies greatly depending upon the solvent in question. And with respect to the "critical point" of adsorption—characterized by a resumed or sharp increase of absorption with increasing concentrations of the solvent—it will be noted that this also varies greatly depending upon the solvent used, and also follows the de-lustering "critical point" by varying differences in concentration.

At such latter concentrations of solvent solutions—with due consideration of the times and temperatures and other conditions and purposes of treatment—the yarn is usually so profoundly altered in its physical structure and composition that it can hardly be regarded as useful as a customary textile or fibrous material.

Accordingly, in general, the safest criterion for textile dyeing purposes is to employ aqueous solutions of the acetate solvents which—at the times and temperatures of the dyeing or other process to be employed—will effect an increase of absorption not exceeding the initial critical point—i. e., that with respect to concentration at which a de-lustering of the acetate occurs.

Graphs of the initial or de-lustering critical points for several solvent solutions are plotted against times and temperatures of treatment on the accompanying chart. From this it will be evident that any one of the solutions of the concentrations indicated may be safely employed, with respect to cellulose acetate yarn, without danger of de-lustering the same, under conditions falling below the corresponding lines on the chart.

Of course, as is well known, de-lustering of cellulose acetate yarn (or other acetate textile products) may not be undesirable but actually desirable, from the commercial standpoint. In such cases, the critical point with respect to de-lustering may purposely be reached or exceeded, so that de-lustering is in fact effected upon the surfaces of the cellulose acetate under treatment. But when this is to be done, as will be obvious from the tables above and from the graph just referred to, precautions must be observed in order not to develop conditions of excessive absorption, by applying excessive concentrations, too long periods of time or too high temperatures, with reference to the specific solvent or solvents which are being used.

But, within the limitations of concentration, of the aqueous solutions of cellulose acetate solvents, and of the times and temperatures of treatment as above described, it is found that cellulose acetate products in general and more specifi-

cally cellulose acetate yarns are so conditioned thereby that they may be safely and especially well dyed to substantially any shade desired and to depths of color equal to or greater than those of the Standard Color Card of America, above referred to, which is an accepted standard of dyeing for the dyeing and textile industry of the United States. These dyeings are superior to those heretofore obtained by standard present-day methods in fastness to light, fastness to bleaching and fastness to washing.

With products other than textiles it may well be practicable to ignore the "critical points" with respect to delustering or with respect to increased absorption and thus to apply mild or drastic actions of the solvent solutions at will and dye with acid dyes—and still get effective and fast dyeing, without detriment to the resulting product. But this is not the case with cellulose acetate yarn, fibers or textile materials generally.

It is now further discovered as a part of the present invention that within these limitations of treating cellulose acetate with aqueous solutions containing one or more solvents of cellulose acetate the latter may not only be dyed with acid dyes, but more effectively and uniformly dyed, if further conditions in the dye bath are observed.

In this connection it is thought that the preliminary absorption of solvent solution by the cellulose acetate, in moderate proportions, as above described, is attributable to the summation of three factors: (1) The natural absorptivity by the cellulose molecule of 7-8% by weight of water or aqueous solution; (2) the inclusion of the solvent solution in the interstitial and pore spaces of the cellulose acetate fibers or the like; and (3) the permeation and diffusion of the aqueous solution of solvent throughout the cellulose acetate structure, per se, which remains in solid form but retains the diffused aqueous solvent solution uniformly dispersed therethrough, in the nature of a solid solution—i. e. of the liquid in the solid cellulose acetate.

When the concentration of the solvent solution in such a system is increased to a sufficient degree in any given case, (or its action is enhanced by increased time or temperature of treatment), this solid-liquid phase tends to merge into a liquid-liquid phase in which the cellulose acetate is liquefied. Thereupon the solid acetate tends to swell, because it partially goes into liquid solution, with intermediate dispersion and hydrolysis by the water present, which induces swelling of the structure as a whole. This latter stage, of marked swelling and subsequent liquefaction of the cellulose acetate by the solvent solution, is definitely to be avoided in the conduct of the present invention, especially for the dyeing of textiles—for in such condition the cellulose acetate is unmanageable and loses its intrinsically desirable properties, as already mentioned. In such condition of limited increase of weight by absorption and limited dimensional expansion or shrinkage, however, it would appear that the cellulose acetate is uniformly and completely penetrated by the aqueous solution of its potential solvent, but that dissolution of the acetate thereby is not appreciably effected.

The potential solvents of cellulose acetate are now found to be effective solvents for the dye acids of the acid dyes—even though used in the form of relatively dilute aqueous solutions. Such

solutions are therefore capable both of dissolving such dye acids and also of penetrating and diffusing through the cellulose acetate as above described. Consequently, when in sufficient concentrations, they are competent to dissolve and to carry the dissolved dye acids through the surface and into the cellulose acetate structure, whether the latter is in the form of fiber, fabric, film, or other sheet material.

Nevertheless, under such conditions alone, effective dyeing of the cellulose acetate will not result, for in the subsequent removal of excess dye solution from the surfaces of the cellulose acetate, followed by washing and drying, etc., the distribution ratio of the dissolved dye between the aqueous solution within the acetate and in the exterior wash water, will be variously altered, generally in the direction of removing the diffused dye solution from the cellulose acetate, thus generally leaving a low color value in the material treated. Likewise, the residual dye actually retained by the cellulose acetate will not be fast against subsequent washing.

It is now further found, however, that an acid dye solution may be diffused uniformly into and through the cellulose acetate as thus treated and simultaneously rendered effective to dye and become fast therein, if the dye bath is impressed with a certain degree of acidity—namely, of sufficient concentration to have a pH value between 0.4 and 1.4, and preferably below 1.0 since the washing fastness is decidedly improved by operating below pH 1.0.

It appears to be practically immaterial how this acidity or pH value is obtained. It may be afforded by using a sufficient concentration of an acidic cellulose acetate solvent, per se,—if this does not at the same time exceed the critical

point of de-lustering or swelling the cellulose acetate.

However, using most solvent organic acids alone (i. e., without inorganic acids such as sulphuric) it is impossible to lower the pH below 1.0—that is, below the limiting pH value required for satisfactory washing fastness—without injuring the yarn. Nevertheless, it is possible to depress the pH value below 1.4 with certain solvent organic acids alone, such as formic acid, and thus to obtain satisfactory dyeings where great fastness to washing is not necessary. Such acidity may likewise be provided partly by the acidity of the acetate solvent (such as formic and/or acetic acid) and partly by the addition of a stronger, inorganic acid—such as sulphuric, hydrochloric and phosphoric acids—which apparently in the concentrations necessary for this purpose are without deleterious effect upon the absorption, structural formation or other physical properties of the cellulose acetate fibers or films, but which do, by enhancing the acidity of the dye solution, render it effective to form and to dissolve the dye acid and to diffuse into and dye the cellulose acetate structure uniformly throughout to a fast color, the depth of color depending directly upon the concentration of the dye in the solution. Again, the cellulose acetate solvent may be non-acidic, such as ethylene chlorhydrin, in which case the inorganic acid alone may be relied upon to provide the required pH value.

Using solvent compositions containing an appropriate concentration of cellulose acetate solvent and of mineral acid, in accordance with the foregoing, numerous skeins of cellulose acetate yarn were treated and results obtained in accordance with the following table:

TABLE 5  
Effect of various bath conditions on absorption  
and luster of yarn

(Note.—All acids by volume)

| Concentration and make-up<br>of bath |                 |                                             | Weight<br>before<br>cond. | Treatment<br>bone<br>dry | Weight<br>after<br>treatment | Absorp-<br>tion | Condi-<br>tion of<br>yarn | Running<br>condi-<br>tions |
|--------------------------------------|-----------------|---------------------------------------------|---------------------------|--------------------------|------------------------------|-----------------|---------------------------|----------------------------|
| Acetic<br>(80%)                      | Formic<br>(85%) | H <sub>2</sub> SO <sub>4</sub><br>(20° Be.) |                           |                          |                              |                 |                           |                            |
| Percent                              | Percent         | Percent                                     | 70.91                     | 65.80                    | 101.07                       | 53.60           | OK.                       | Min. °E.<br>30-125         |
| 8.3                                  | 8.3             | 8.3                                         | 70.01                     | 64.96                    | 99.27                        | 52.95           | OK.                       | 60-125                     |
| 8.3                                  | 8.3             | 8.3                                         | 69.80                     | 64.76                    | 97.36                        | 50.40           | OK.                       | 120-125                    |
| 8.3                                  | 8.3             | 8.3                                         | 70.41                     | 65.34                    | 98.53                        | 50.80           | OK.                       | 180-125                    |
| 8.3                                  | 8.3             | 8.3                                         | 69.98                     | 64.93                    | 97.71                        | 50.50           | OK.                       | 240-125                    |
| 8.3                                  | 8.3             | 8.3                                         | 73.19                     | 67.93                    | 107.66                       | 58.34           | SI.                       | 360-125                    |
| 8.3                                  | 8.3             | 8.3                                         | 37.20                     | 35.39                    | 54.36                        | 53.60           | OK.                       | 30-80                      |
| 8.3                                  | 8.3             | 8.3                                         | 42.80                     | 40.05                    | 62.49                        | 56.10           | OK.                       | 30-120                     |
| 8.3                                  | 8.3             | 8.3                                         | 62.12                     | 58.81                    | 89.04                        | 51.42           | Bad                       | 30-140                     |
| 8.3                                  | 8.3             | 8.3                                         | 69.62                     | 68.00                    | 92.34                        | 39.00           | Bad                       | 30-160                     |
| 8.3                                  | 8.3             | 8.3                                         | 64.70                     | 60.04                    | 87.72                        | 46.00           | Bad                       | 30-180                     |
| 2.5                                  | 2.5             | 8.3                                         | 73.41                     | 69.30                    | 97.55                        | 40.80           | OK.                       | 30-125                     |
| 5                                    | 5               | 8.3                                         | 60.21                     | 57.19                    | 82.38                        | 44.10           | OK.                       | 30-125                     |
| 7.5                                  | 7.5             | 8.3                                         | 69.83                     | 66.19                    | 95.10                        | 43.80           | OK.                       | 30-125                     |
| 10                                   | 10              | 8.3                                         | 43.20                     | 41.20                    | 60.46                        | 47.10           | Bad                       | 30-125                     |
| 2.5                                  | 2.5             | 2.5                                         | 70.48                     | 66.82                    | 99.96                        | 49.60           | OK.                       | 30-125                     |
| 5                                    | 5               | 5                                           | 71.32                     | 67.61                    | 101.04                       | 49.50           | OK.                       | 30-125                     |
| 7.5                                  | 7.5             | 7.5                                         | 69.37                     | 65.76                    | 98.50                        | 42.82           | OK.                       | 30-125                     |
| 10                                   | 10              | 10                                          | 70.63                     | 66.96                    | 100.17                       | 49.62           | SI.                       | 30-125                     |
| 5                                    | 2.5             | 68.98                                       | 64.02                     | 94.15                    | 47.06                        | OK.             | 30-125                    |                            |
| 10                                   | 5               | 70.45                                       | 65.38                     | 94.69                    | 44.98                        | OK.             | 30-125                    |                            |
| 15                                   | 7.5             | 69.67                                       | 64.64                     | 95.90                    | 48.36                        | OK.             | 30-125                    |                            |
| 20                                   | 10              | 70.65                                       | 65.46                     | 101.68                   | 55.33                        | SI.             | 30-125                    |                            |
| 5                                    | 8.3             | 66.29                                       | 61.51                     | 90.51                    | 47.15                        | OK.             | 30-125                    |                            |
| 10                                   | 8.3             | 47.98                                       | 45.68                     | 67.40                    | 47.70                        | OK.             | 30-125                    |                            |
| 15                                   | 8.3             | 49.49                                       | 47.04                     | 68.61                    | 45.82                        | OK.             | 30-125                    |                            |
| 20                                   | 8.3             | 41.88                                       | 39.30                     | 59.38                    | 49.20                        | SI.             | 30-125                    |                            |
| 5                                    | 2.5             | 43.56                                       | 41.44                     | 60.61                    | 45.78                        | OK.             | 30-125                    |                            |
| 10                                   | 5               | 61.26                                       | 48.70                     | 71.41                    | 46.68                        | OK.             | 30-125                    |                            |
| 15                                   | 7.5             | 48.37                                       | 46.00                     | 68.81                    | 49.58                        | SI.             | 30-125                    |                            |
| 20                                   | 10              | 69.49                                       | 64.47                     | 97.45                    | 51.19                        | Bad             | 30-125                    |                            |
| 5                                    | 8.3             | 71.60                                       | 68.44                     | 94.84                    | 42.75                        | OK.             | 30-125                    |                            |
| 10                                   | 8.3             | 71.81                                       | 66.64                     | 102.54                   | 53.87                        | OK.             | 30-125                    |                            |
| 15                                   | 8.3             | 71.90                                       | 66.72                     | 103.01                   | 54.18                        | OK.             | 30-125                    |                            |
| 20                                   | 8.3             | 71.29                                       | 68.15                     | 101.35                   | 53.14                        | OK.             | 30-125                    |                            |

In each case the yarn was conditioned to 60% humidity and calculated to bone dry weight, by analysis of representative skeins treated, and then freed from surplus moisture after treatment and weighed. These several weighings were all recorded and show that (with one exception) all of the treatments resulted in increased absorption of the solvent solution or water, by the yarn, in excess of 41.9% by weight.

In thus removing the surplus moisture from the skeins, a centrifuge was used having a basket of  $5\frac{1}{4}$ " inside diameter and inside height 2" to the flanged top, which was  $\frac{1}{2}$ " wide. The perforations in the side walls were  $\frac{1}{4}$ " diameter. The basket was first loaded, with three skeins as used in these experiments, and then brought up to full speed in five seconds, held at full speed of 4300 R. P. M. for twenty seconds, and finally allowed to coast to rest, usually taking about thirty seconds.

From these results it is demonstrated that increased concentration of the solvent, and accompanying increased absorptivity of the yarn, progress together.

Likewise, increased depth of shade in the yarn is effected by the dye bath, as thus induced by the presence of solvent, and full shades may be obtained in the yarn thereby. When the time, temperature or concentration of the solution exceeds the critical point the yarn is de-lustered, or even partially hydrated. For some purposes, as already noted, such de-lustering may be desirable, but if these conditions are carried too far the yarn or textile may be partially or completely decomposed so that the product is ruined. In such case the decomposed yarn may and usually does retain the acid dye therein, but the procedure is not one which can be successfully applied to cellulose acetate yarns, fabrics, or other textiles.

It is believed that the free dye acid, which is liberated at the low pH values hereinabove recommended, is also thereby maintained in free acid condition and dissolved in the dye bath solution in this form. Also that these pH values, in the presence of the acetate solvent solution, condition the hydrolyzed cellulose acetate throughout its structure, to a similar acidity and that under these acidic conditions the cellulose acetate and dissolved free dye acid react to form an insoluble, colored reaction product. Subsequent dilution and washing with water will dissolve out and remove both the acetate solvent and the acid, but not the dye acid which has thus become associated with and within the solid cellulose acetate structure. That this is the case is demonstrated by the fact that while the acetate solvent which has also dissolved the dye and carried it into and throughout the cellulose acetate structure is still present both outside of and throughout the acetate fiber it does not appear to be able to dissolve the dye and remove it from within the fiber structure. At least the partition ratio of the dye in the solution and within the acid-dyed cellulose acetate fiber is different from the partition ratio of the dye between the solution and the undyed cellulose acetate fiber. In this respect, the results are quite different from those which obtain when cellulose acetate is treated with a solvent solution of like concentra-

tion and containing an acid dye in solution, but having a high pH value. Under such conditions, while the dye will dissolve and permeate the structure of the cellulose acetate fiber it will also migrate outwardly into the surrounding solution, upon dilution, washing, and the like.

Another advantageous feature of the present procedure is that the yarn may be dyed in package form, by pressure dyeing—i. e., by pumping the dye solution through the wound yarn—much more readily than by previously known methods of dyeing acetate. In the present process, it is believed that the liberated dye acid is completely dissolved to form a true or molecular solution in the dye bath which consequently passes both between and into the cellulose acetate fibers and structure without segregation until within the cellulose acetate structure of the yarn and that here it becomes permanently and uniformly fixed and insoluble.

By thus permitting the dyeing operation to be effected with dye acids and by the pressure method, it is also made possible to use short liquor ratios, with consequent reduction in the amounts of dye bath compositions required and the residual amounts of solution left over after each given dyeing operation has been completed. For example, liquor ratios as low as 3 to 1 may be used as compared to formerly required ratios of 20-40 to 1.

The application of the invention will be exemplified by the following specific procedures which are representative of its fundamental aspects of utility in the art of dyeing cellulose acetate with acid dyes.

The following uniform dyeing procedure was followed in each case shown in Tables 6 to 10:

Skeins of acetate yarn were wet out and secured in the ordinary way. They were then entered into the dye bath. Up to this point all skeins were treated alike. In all cases the weight of the dye bath was 15 times that of the yarn, and the dye concentration was 0.15% on the bath. The temperature of the bath was maintained at 125° F. and the time in the bath was 30 minutes. After removal from the bath, the skeins were gently wrung out; they were then rinsed, soaped, rinsed, extracted, and dried in the usual manner. Temperature of the rinsing and soaping baths was about 125° F.

In commercial practice the procedure is similar. However the dye concentration will be varied to meet the shade desired and the soaping temperature can be increased to as high as 180° F. depending on fastness requirements.

Examples of the dyes which have been thus employed may be numbered as follows:

TABLE 6

- #1. Wool Fast Blue BLA Extra New Color Index No. 833.
- #2. Azo Rubinol 3 GP. (Patented) Sandoz Chemical Works Inc.
- #3. Alizarine Cyanine Green GHA Extra Color Index No. 1078.
- #4. Fast Silk Yellow G (Geigy Company).
- #5. Milling Red SWG Color Index No. 430.

TABLE 7

pH determinations of solutions having different amounts of acids corresponding to those of dye bath solutions

| Code letter <sup>1</sup><br>(if any) | Formic acid<br>85% | Acetic acid<br>80% | Sulphuric acid<br>20° Bé. | pH values— |            |
|--------------------------------------|--------------------|--------------------|---------------------------|------------|------------|
|                                      |                    |                    |                           | At 72° F.  | At 125° F. |
|                                      |                    |                    |                           |            |            |
|                                      | Per cent           | Per cent           | Per cent                  |            |            |
|                                      | 1                  | 1                  | 1                         | 1.7        | 1.3        |
|                                      | 2                  | 2                  | 2                         | 1.4        | 1.1        |
|                                      | 3                  | 3                  | 3                         | 1.3        | 0.9        |
| X                                    | 5                  | 5                  | 5                         | 1.15       | 0.7        |
| H                                    | 8½                 | 8½                 | 8½                        | 0.85       | 0.4        |
| W                                    | 10                 | 10                 | 10                        | 0.75       | 0.3        |
| I                                    | 11                 | 11                 | 11                        | 0.7        | 0.3        |
|                                      | 5                  |                    |                           | 2.5        | 2.3        |
|                                      | 10                 |                    |                           | 2.35       | 2.15       |
|                                      | 15                 |                    |                           | 2.25       | 2.0        |
| F                                    | 16½                |                    |                           | 2.2        | 2.0        |
| D                                    | 25                 |                    |                           | 2.0        | 1.85       |
| M                                    | 33                 |                    |                           | 1.9        | 1.7        |
| B                                    | 16½                |                    | 8½                        | 0.9        | 0.5        |
| K                                    | 22                 |                    | 11                        | 0.8        | 0.4        |
| G                                    |                    |                    | 25                        | 0.6        | 0.1        |
| N                                    |                    |                    | 33                        | 0.5        | 0.1        |
| V                                    | 8½                 | 8½                 |                           | 1.7        | 1.45       |
| P                                    | 5                  |                    |                           | 1.9        | 1.7        |
| Q                                    | 10                 |                    |                           | 1.7        | 1.5        |
| R                                    | 15                 |                    |                           | 1.5        | 1.3        |
| E                                    | 16½                |                    |                           | 1.45       | 1.2        |
| C                                    | 25                 |                    |                           | 1.3        | 1.0        |
| L                                    | 33                 |                    |                           | 1.05       | 0.8        |
| S                                    | 5                  |                    | 10                        | 0.85       | 0.55       |
| T                                    | 10                 |                    | 10                        | 0.8        | 0.5        |
| U                                    | 15                 |                    | 10                        | 0.7        | 0.4        |
| A                                    | 16½                |                    | 8½                        | 0.7        | 0.4        |
| J                                    | 22                 |                    | 11                        | 0.6        | 0.2        |

<sup>1</sup> The code letters are those appearing in the specification below.  
Parts are by volume.

Inasmuch as the acidity here involved is so high, colorimetric methods would not be satisfactory. Accordingly the values given in the table were determined electrometrically, using a Coleman Electrometer No. 3. Similar commercial apparatus could be used instead.

The pH readings at 72° F. were taken with both the room temperature and the solution temperature at 72° F., in the conventional manner, the apparatus being standardized against a pH value of 1.00 for 0.1 N HCl at 72°. The standard against which the set was calibrated was 0.1 N HCl, which was taken to have a pH value of 1.00 at 125° F. This was then further checked against 1.0 N HCl at 125° F. whose theoretical pH is 0 and the actual pH value was found to be less than 0.001.

In taking the pH readings of the solutions at 125° F. precautions were observed to correct for the temperature difference between the solutions and the room. In making these pH measurements and those of the solutions, the temperature compensator of the set was placed in the bath kept at 125° F. and the 0.1 N HCl was kept by a temperature bath arrangement at 125° F. in the sample cup. The assymetry potential knob was adjusted until the set balanced at pH=1.00 when testing the 0.1 N HCl. The calomel electrode was at room temperature during all of the measurements. The solutions being tested at 125° F. were introduced at that temperature and maintained at that temperature by means of a water bath. Readings were taken at once and again after various intervals from 1 to 5 minutes. The pH variation between the different times of readings was generally less than 0.01 and never over 0.02.

TABLE 8

Quantitative comparison of color depth obtained with dyes of Table 6 used in dye baths having amounts of acids and pH values corresponding to those of Table 7

[An arbitrary scale is taken for each color, from 0 to 20, the darkest shade being designated by 20 and absence of any dyeing designated by 0.]

| Run No. | #1 Wool Fast Blue | #2 Azo Rubinol | #3 Alizarine Cyanine Green | #4 Fast Silk Yellow | #5 Milling Red |
|---------|-------------------|----------------|----------------------------|---------------------|----------------|
| 15      |                   |                |                            |                     |                |
| A       | 15                | 19             | 12                         | 17                  | 14             |
| B       | 16                | 15             | 14                         | 17                  | 13             |
| C       | 19                | 18             | 20                         | 18                  | 18             |
| D       | 12                | 11             | 15                         | 17                  | 10             |
| E       | 10                | 13             | 13                         | 17                  | 12             |
| F       | 6                 | 8              | 10                         | 16                  | 6              |
| G       | 2                 | 3              | 4                          | 6                   | 1              |
| H       | 18                | 17             | 16                         | 19                  | 14             |
| I       | 20                | 20             | 18                         | 20                  | 20             |
| J       |                   |                |                            |                     | 18             |
| K       |                   |                |                            |                     | (25)           |
| L       |                   |                |                            |                     | Above (20)     |
| M       |                   |                |                            |                     | 15             |
| N       |                   |                |                            |                     | 1              |
| P       | 4                 | 5              | 5                          | 9                   | 4              |
| Q       | 7                 | 9              | 9                          | 16                  | 8              |
| R       | 12                | 13             | 13                         | 17                  | 12             |
| S       | 5                 | 10             | 6                          | 8                   | 5              |
| T       | 8                 | 15             | 9                          | 16                  | 11             |
| U       | 15                | 19             | 12                         | 17                  | 14             |

It may be remarked, with reference to the data in the above table, that those dye bath compositions containing sulphuric acid and no organic acid solvent, are not to be considered as within the present invention. Sulphuric acid is not, per se, a solvent of cellulose acetate, and the dyeing results obtained are manifestly too low for consideration as being satisfactory. Likewise solutions containing 5% of formic acid alone (and without sulphuric acid) demonstrate that this concentration is at the threshold value with respect to its action toward cellulose acetate, and also of insufficient acidity (pH 1.8) per se, to provide the required pH (1.4) for imparting a fast dyeing effect to the cellulose acetate yarn.

It is also found that results similar to those given above may be obtained by using comparable amounts of other inorganic acids, instead of sulphuric acid—such as hydrochloric acid and phosphoric acid—which are actually equivalent in the ratio 1:2:5 by weight, of 100% hydrochloric, sulphuric and phosphoric acids respectively. Thus, using Azo Rubinol (#2) under conditions corresponding to A, B, G and H, the following comparative color values were obtained in dyeing:

TABLE 9

| Composition | Sulphuric (20° Bé.) | Hydrochloric (13%) | Phosphoric (60%) |
|-------------|---------------------|--------------------|------------------|
| A           | 19                  | 19                 | 17               |
| B           | 15                  | 14                 | 11               |
| G           | 3                   | 2                  | 2                |
| H           | 17                  | 18                 | 15               |

Again, using lactic acid in place of the formic or acetic acids of the above tables yields effective results, the lactic acid being a decidedly less active solvent:

TABLE 10

| Lactic acid (85% strength) | Wool Fast Blue | Azo Rubinol | Milling Red |
|----------------------------|----------------|-------------|-------------|
| 25%<br>Plus 8.3% sulphuric | 8              | 9<br>10     | 7           |

In the commercial application of the process of the invention, especially for the dyeing of cellulose acetate yarns, it is particularly desirable to carry it out by the pressure method of forcing the dyeing solution through the yarn while it is in wound or package form. For this purpose, the apparatus described in U. S. Patent No. 2,125,937 is entirely suitable and convenient to use.

The yarn is wound in packages of about a pound and these are loaded upon hollow, perforated spindles, with a separator plate between the end of each package and the end of the one next to it. The full spindles (holding eight packages on each) are loaded onto the removable machine carrier.

In a given case, using acetate yarn of 200 denier, 64 filaments, 3 turns per inch, the full load may amount to approximately 1000 pounds. This is lowered into the dye machine and scoured with soap for 15 minutes at 160° F. to remove the softening oils on the natural yarn. The charge is then rinsed free of soap, extracted in a centrifuge, and dried at 150° F. for 20 hours.

The dye bath is prepared in the following manner.

4000 lbs. total weight of bath, are made up as follows:

|       |                                                                                                        |
|-------|--------------------------------------------------------------------------------------------------------|
| 1000  | lbs. water                                                                                             |
| 333.3 | lbs. of 85% formic acid                                                                                |
| 333.3 | lbs. of 84% acetic acid                                                                                |
| 333.3 | lbs. of 20° Bé. sulphuric acid solution<br>(or 85 lbs. 66° Bé. sulphuric acid<br>and 248.3 lbs. water) |
| 2000  | lbs. water (180° F.) to dissolve the following dyes.                                                   |
| 44.0  | lbs. (4.4% of weight of yarn) Alizarine<br>Cyanine Green GHA extra                                     |
| 12.0  | lbs. (1.2% of weight of yarn) Fast Silk<br>Yellow G                                                    |
| 2.5   | lbs. (0.25% of weight of yarn) Wool Fast<br>Blue BLA                                                   |

The dyes are dissolved in the 2000 lbs. of hot water and the resulting solution is put into the dyeing machine which already contains the 2000 lbs. of solvent solution, made up of the constituents, as listed above, and the two solutions are intimately mixed.

The yarn is then entered into the dye bath, and the bath is pumped through the packages for 30 minutes, at about 80° F. The temperature is then gradually increased to 125° F. and the dye bath circulated for 90 minutes. The dye bath is then dropped and the yarn is rinsed with three successive water baths to remove the acids. The yarn is then soaped twice at 170° F., rinsed, and softened in an oil emulsion rinse. The packages are then extracted by centrifuging and dried. The yarn is inspected for defects, and may be wrapped, and shipped in the package form.

I claim:

1. Method of dyeing cellulose acetate with an acid dye, comprising the step of treating the acetate with an acid dye and with an aqueous solution of an organic solvent thereof having a concentration between its threshold value and its

critical point, with reference to the absorption of the material treated, and an inorganic acid.

2. Method of dyeing cellulose acetate with an acid dye, comprising the step of treating the acetate with an acid dye and with an aqueous solution of an organic acid solvent thereof having a concentration between its threshold value and its critical point, with reference to the absorption of the material treated.

10 3. Method of dyeing cellulose acetate with an acid dye, comprising the step of treating the acetate with an acid dye and with an aqueous solution of an organic solvent thereof having a concentration between its threshold value and its critical point, with reference to the de-lustering of the material treated, and an inorganic acid.

20 4. Method of dyeing cellulose acetate with an acid dye, comprising the step of treating the acetate with an acid dye and with an aqueous solution of an organic acid solvent thereof having a concentration between its threshold value and its critical point, with reference to the de-lustering of the material treated.

25 5. Method of dyeing cellulose acetate, comprising treating the same with an aqueous solution of one of its organic solvents having a concentration between its threshold value and its critical point, with reference to the absorption of the material treated, and containing an acid dye or dye acid, at a pH value below 1.4.

30 6. Method of dyeing cellulose acetate, comprising treating the same with an aqueous solution of one of its organic acid solvents having a concentration between its threshold value and its critical point, with reference to the absorption of the material treated, and containing an acid dye or dye acid, at a pH value below 1.4.

35 7. Method of dyeing cellulose acetate, comprising treating the same with an aqueous solution of one of its organic solvents having a concentration between its threshold value and its critical point, with reference to the de-lustering of the material treated, and containing an acid dye or dye acid, at a pH value below 1.4.

40 8. Method of dyeing cellulose acetate, comprising treating the same with an aqueous solution of one of its organic acid solvents having a concentration between its threshold value and its critical point, with reference to the de-lustering of the material treated, and containing an acid dye or dye acid, at a pH value below 1.4.

45 9. Method of dyeing cellulose acetate, comprising the step of circulating through a mass of the same, under pressure, a dye bath composition containing an aqueous solution of an organic solvent of the acetate having a concentration between its threshold value and its critical point with reference to absorption, and a dye acid in solution therein, and characterized by a pH value below 1.4.

50 10. Method of dyeing cellulose acetate, comprising the step of circulating through a mass of the same, under pressure, a dye bath composition containing an aqueous solution of an organic solvent of the acetate having a concentration between its threshold value and its critical point with reference to delustering, and a dye acid in solution therein, and characterized by a pH value below 1.4.

55 11. Method of dyeing cellulose acetate, comprising the steps of treating successive charges of the same in a dye bath composition containing an aqueous solution of an organic solvent of the acetate, having a concentration between its

threshold value and its critical point with reference to absorption, and a dye acid in solution therein, and characterized by a pH value below 1.4, and maintaining said dye bath composition by additions of the dye acid thereto.

12. Method of dyeing cellulose acetate, comprising the steps of treating successive charges of the same in a dye bath composition containing an aqueous solution of an organic solvent of the acetate, having a concentration between its threshold value and its critical point with reference to de-lustering, and a dye acid in solution therein, and characterized by a pH value below 1.4, and maintaining said dye bath composition by additions of the dye acid thereto.

13. A composition for use in dyeing cellulose acetate with acid dyes, characterized by containing an aqueous solution of a dye acid and of an organic solvent of cellulose acetate, having a concentration between its threshold value and its critical point with reference to absorption at the temperatures and for the period of dyeing in question, and an inorganic acid.

14. A composition for use in dyeing cellulose acetate with acid dyes, characterized by containing an aqueous solution of a dye acid and of an organic acid solvent of cellulose acetate, having a concentration between its threshold value and its critical point with reference to absorption at the temperatures and for the period of dyeing in question.

15. A composition for use in dyeing cellulose acetate with acid dyes, characterized by containing an aqueous solution of a dye acid and of an organic solvent of cellulose acetate, having a concentration between its threshold value and its critical point with reference to de-lustering, at the temperatures and for the period of dyeing in question, and an inorganic acid.

16. A composition for use in dyeing cellulose acetate with acid dyes, characterized by containing an aqueous solution of a dye acid and of an organic acid solvent of cellulose acetate, having a concentration between its threshold value and its critical point with reference to de-lustering at the temperatures and for the period of dyeing in question.

17. A dye bath composition for dyeing cellulose acetate with acid dyes, characterized by containing an aqueous solution of an organic solvent of cellulose acetate, having a concentration between its threshold value and its critical point, with reference to absorption, a dye acid, and a pH value below 1.4.

18. A dye bath composition for dyeing cellulose acetate with acid dyes, characterized by

containing an aqueous solution of an organic acid solvent of cellulose acetate, having a concentration between its threshold value and its critical point, with reference to absorption, a dye acid, and a pH value below 1.4.

19. A dye bath composition for dyeing cellulose acetate with acid dyes, characterized by containing an aqueous solution of an organic solvent of cellulose acetate, having a concentration between its threshold value and its critical point, with reference to de-lustering, a dye acid, and a pH value below 1.4.

20. A dye bath composition for dyeing cellulose acetate with acid dyes, characterized by containing an aqueous solution of an organic acid solvent of cellulose acetate, having a concentration between its threshold value and its critical point, with reference to de-lustering, a dye acid, and a pH value below 1.4.

21. Method of dyeing cellulose acetate with an acid dye, comprising treating the acetate with an acid dye and with an aqueous solution of an inorganic acid and an organic acid solvent for said cellulose acetate, said solution having a concentration between its threshold value and its critical point with reference to the absorption of the material treated.

22. Method of dyeing cellulose acetate with an acid dye, comprising treating the acetate with an acid dye and with an aqueous solution of an inorganic acid and an organic acid solvent for said cellulose acetate, said solution having a concentration between its threshold value and its critical point with reference to the de-lustering of the material treated.

23. A composition for use in dyeing cellulose acetate with acid dyes, characterized by containing an aqueous solution of a dye acid, an inorganic acid and an organic acid solvent of cellulose acetate, said solution having a concentration between its threshold value and its critical point with reference to absorption, at the temperatures and for the period of dyeing in question.

24. A composition for use in dyeing cellulose acetate with acid dyes, characterized by containing an aqueous solution of a dye acid, an inorganic acid and an organic acid solvent of cellulose acetate, said solution having an effective concentration with reference to the material treated between its threshold value and its critical point with reference to de-lustering, at the temperatures and for the period of dyeing in question.

LUIGI C. GALATIOTO.